

# UNITED STATES PATENT OFFICE.

ALEXANDRE N. DUBOIS, OF PHILADELPHIA, PENNSYLVANIA.

## DYEING ANILINE-BLACK.

SPECIFICATION forming part of Letters Patent No. 283,220, dated August 14, 1883.

Application filed April 14, 1883. (No specimens.)

*To all whom it may concern:*

Be it known that I, ALEXANDRE N. DUBOIS, of Philadelphia, in the county of Philadelphia and State of Pennsylvania, have invented certain new and useful Improvements in the Process of Dyeing Aniline-Black, of which the following is a specification.

My invention relates to the dyeing of cotton, cloth, yarn, and vegetable fabrics through the medium of aniline; and the object of my invention is to obtain economy and simplicity in the dyeing, the production on the materials of an indelible black, and to greatly shorten the time required to dye the goods over the processes now in use.

My dyeing-bath is composed as follows: I take of the weight of the material to be dyed about eight hundred per cent. of tepid water, and in it I dissolve eight per cent. of aniline salt, four per cent. hydrochloric acid at 22° Baumé, eight per cent. sulphuric acid at 66° Baumé, twelve per cent. sulphate of soda, and fourteen percent. bichromate of potash. This bath is thoroughly moved or stirred, and the

fabrics to be dyed are placed in it and moved around or worked from forty to fifty minutes, then taken out, washed well in cold water, and dried and finished in the usual manner. This bath is adapted for dyeing cotton, yarn, cloth, and textile fabrics of all kinds.

I do not limit myself to the proportions specified above, as they may be varied to suit the different requirements of the different substances to be dyed.

Having thus described my invention, I claim—

The process of dyeing cotton, cloth, yarn, and fabrics of all kinds, consisting in immersing them in a bath composed of water, aniline salt, hydrochloric acid, sulphuric acid, sulphate of soda, and bichromate of potash, in or about the proportions specified.

In testimony whereof I affix my signature in presence of two witnesses.

ALEXANDRE N. DUBOIS.

Witnesses:

CHRISTOPHER FALLON,  
GEO. DENGLER.